# EUROPEAN PATENT APPLICATION

(11) **EP 0 282 262 A1**
(43) Date of publication of application: **14.09.1988**
(21) Application number: 88302002.6
(22) Date of filing: 08.03.1988
(51) Int. Cl.: C10L 9/00

(54) **Method for improving the density of coke**

(30) Priority: 09.03.1987 US 23737
(71) Applicant: Conoco Inc., Ponca City Oklahoma 74603 (US)
(72) Inventor: Shouse, James W., Blackwell Oklahoma 74631 (US); Newman, Bruce A., Ponca City Oklahoma 74604 (US); Johnson, Eric S., Minato-ku Tokyo (JP)
(74) Representative: Woodman, Derek

(57) **Abstract**

The density of calcined coke is improved by contacting green (uncalcined) coke with coker feedstock prior to calcining the green coke.

## Description

### Background and Summary of the Invention

There is an increasing demand for high quality premium coke for the manufacture of large graphite electrodes for use in electric arc furnaces employed in the steel industry. A number of properties are of importance in characterizing the quality of graphite electrodes. One such property is density. Usually the higher the density the better the electrode. Users of premium coke continuously seek graphite materials having higher densities. Even a small change in density can have a substantial effect on large electrode properties.

Premium coke is manufactured by delayed coking in which heavy hydrocarbon feedstocks are converted to coke and lighter hydrocarbon products. In the process the heavy hydrocarbon feedstock is heated rapidly to cracking temperatures and is fed into a coke drum. The heated feed soaks in the drum in its contained heat which is sufficient to convert it to coke and cracked vapors. The cracked vapors are taken overhead and fractionated with the fractionator bottoms being recycled to the feed if desired. The coke accumulates in the drum until the drum is filled with coke at which time the heated feed is diverted to another coke drum while the coke is removed from the filled drum. After removal the coke is calcined at elevated temperatures to remove volatile materials and to increase the carbon to hydrogen ratio of the coke.

In the manufacture of large graphite electrodes, calcined premium coke particles obtained from the delayed coking process are mixed with pitch and then baked at elevated temperatures to carbonize the pitch.

According to this invention, calcined coke having increased density is produced by contacting the coke prior to calcining with coker feedstock and thereafter carrying out the calcining operation. In one embodiment the process is employed to obtain premium coke of increased density for use in the manufacture of electrodes employed in the production of steel.

### Prior Art

U. S. Patent No. 2,502,183 discloses making a dense carbon by mixing carbon aggregate, coke "flour", and pitch and hot molding the mixture to produce a dense carbon article. The patent also discloses production of carbon electrodes and other articles by hot molding a pulverized mixture containing a major proportion of carbonaceous residue together with a minor proportion of more completely carbonized material such as fully calcined petroleum coke. The only coke "flour" disclosed in the patent is calcined petroleum coke.

U. S. Patent 4,105,501 discloses a process for the manufacture of metallurgical formed coke by carbonizing briquettes made by forming an outer envelope of a bituminous material over coal fines. Bituminous materials disclosed are coal tar, coal tar pitch, emulsified coal tar pitch, asphalt, modified asphalt, and heat treated asphalt.

U. S. Patent No. 4,483,840 discloses a process in which pellets resulting from the agglomeration of anthracite or other coal fines with a binder based on pitch and/or tar are subjected to an oxidation treatment at an elevated temperature and are thereafter calcined at a still higher temperature. Resulting pellets may be used for the manufacture of all types of carbonaceous paste, electrodes and carbonaceous blocks for the linings of furnaces or electrolysis cells.

### Brief Description of the Drawing

The drawing is a schematic flow diagram of a premium delayed coker which illustrates one embodiment of the invention.

### Detailed Description of the Invention

The fresh feedstocks used in the preparation of premium coke are heavy aromatic mineral oil fractions. These feedstocks can be obtained from several sources including petroleum, shale oil, tar sands, coal and the like. Specific feedstocks include decant oil, also known as slurry oil or clarified oil, which is obtained from fractionating effluent from the catalytic cracking of gas oil and/or residual oils. Another feedstock which may be employed is ethylene or pyrolysis tar. This is a heavy aromatic mineral oil which is derived from the high temperature thermal cracking of mineral oils to produce olefins such as ethylene. Another feedstock is vacuum resid which is a heavy residual oil obtained from flashing or distilling a residual oil under a vacuum. Still another feedstock is vacuum gas oil which is a lighter material obtained from flashing or distillation under vacuum. Thermal tar may also be used as a feedstock. This is a heavy oil which may be obtained from fractionation of material produced by thermal cracking of gas oil or similar materials. Heavy premium coker gas oil is still another feedstock and is the heavy oil obtained from liquid products produced in the coking of oils to premium coke. Gas oil from coking operations other than premium coking may also be employed as a feedstock. Virgin atmospheric gas oil may also be used as a feedstock. This is gas oil produced from the fractionation of crude oil under atmospheric pressure or above. Another feedstock which may be used is extracted coal tar pitch. Any of the preceding feedstocks may be used singly or in combination. In addition any of the feedstocks may be subjected to hydrotreating, heat soaking, thermal cracking, or a combination of these steps, prior to their use for the production of premium grade coke.

Any of the above feedstocks may be used to contact the green (uncalcined) premium coke in carrying out the process of the invention. Preferred are feedstocks which provide high yields of coke, such as thermal tars, decant oils, pyrolysis tars and various types of pitches. The green coke may be contacted with a portion of the same feedstock used in the preparation of the coke, or, if desired a different feed material may be used for this purpose.

All types of green premium coke are applicable to process of the invention. Thus green coke prepared from any of the conventional coke feedstocks may be used. The largest improvements in coke density occur in instances where the VBD (vibrated bulk density) of the calcined coke is less than about 0.77 g/cc (for 3×6 particles). However, the process is applicable to cokes having lesser or greater density.

Referring now to the drawing, feedstock is introduced into the coking process via line 2. The feedstock which in this instance is a thermal tar is heated in furnace 3 to temperatures normally in the range of about 850°F to about 1100°F and preferably between about 900°F to about 975°F. A furnace that heats the thermal tar rapidly to such temperatures such as a pipestill is normally used. The thermal tar exits the furnace at substantially the above indicated temperatures and is introduced through line 4 into the bottom of coke drum 5 which is maintained at a pressure of between about 15 and about 200 psig. The coke drum operates at a temperature in the range of about 800°F to about 1000°F, more usually between about 820°F and about 950°F. Inside the drum the heavy hydrocarbons in the thermal tar crack to form cracked vapors and premium coke. Cracked vapors are continuously removed overhead from coke drum 5 through line 6. The coke accumulates in the drum until it reaches a predetermined level at which time the feed to the drum is shut off and switched to a second coke drum 5a wherein the same operation is carried out. This switching permits drum 5 to be taken out of service, opened and the accumulated coke removed therefrom using conventional techniques. The coking cycle may require between about 16 and about 60 hours but more usually is completed in about 24 to about 48 hours.

The vapors that are taken overhead from the coke drums are carried by line 6 to a fractionator 7. In the fractionator the vapors are separated into a C₁ - C₃ product stream 8, a gasoline boiling range product stream 9, a light gas oil product stream 10 and a premium coker heavy gas oil taken from the fractionator via line 11. As indicated previously the premium coker heavy gas oil from the fractionator may be recycled at the desired ratio to the coker furnace through line 12. Any excess net bottoms may be subjected to conventional residual refining techniques if desired.

Green coke is removed from coke drums 5 and 5a through outlets 13 and 13a, respectively, and is introduced via 14 to coke soaker 16. The coke soaker comprises a tank or container 17 of liquid thermal tar feedstock and a continuous flexible belt 15 a portion of which is immersed in the tank of feedstock. The green coke is introduced on the flexible belt 15 and passes downwardly through the bath of feedstock. The coke soaked with feedstock then passes upwardly on the belt and out of the soaker and is introduced to calciner 19. Any excess of feedstock on the coke leaving the soaker flows down the belt and back into tank 17. As feedstock is consumed in the coke soaker, additional material is introduced through line 18 in a sufficient quantity to maintain the level of feedstock in tank 17. The amount of feedstock taken up by the coke will vary depending on the particular coke and the feedstock used. Usually feedstock consumption is between about 2 and about 20 percent by weight based on the green coke.

In addition to the method disclosed other conventional procedures may be used for contacting the coke with feedstock. For example, liquid feedstock may be sprayed on the coke or, if the feedstock is a solid at ambient temperature, coke may be passed through finely divided feedstock powder.

Coke is usually removed from the coke drums with a high velocity jet of water. As a result the coke is cooled rapidly and by the time it enters the coke soaker 16 it has reached a relatively low temperature. This is important since contacting hot coke in a bath of liquid feedstock could result in boiling and vaporization of the liquid which would defeat the purpose of the invention. It is not necessary however that the coke be reduced to room temperature. A somewhat heated coke can be advantageous in the wetting process.

The flexible belt 15 may become fouled with liquid feedstock and coke particles over a period of time. It may be cleaned by washing or spraying with a lighter hydrocarbon fraction, or heated feedstock may be used for this purpose.

In calciner 19 the green coke soaked with feedstock is subjected to elevated temperatures to remove volatile materials and to increase the carbon to hydrogen ratio of the coke. Calcination is carried out at temperatures in the range of between about 2000°F and about 3000°F and preferably between about 2400 and about 2600°F. The coke is maintained under calcining conditions for between about one half hour and about ten hours and preferably between about one and about three hours. The calcining temperature and the time of calcining will vary depending on the properties of the coke desired. Calcined premium coke of increased density which is suitable for the manufacture of large graphite electrodes is withdrawn from the calciner through outlet 20.

The following examples illustrate the results obtained in carrying out the invention.

### Example 1

A mixture of thermal tar and decant oil was coked in a delayed coker at 28 psig and 878°F. The coking cycle was 44 hours. A sample of the resulting green coke was covered in a beaker for 15 minutes by a mixture of chloroform and 900°F+ solvent soluble coal tar pitch (2 parts chloroform: 1 part pitch). The chloroform/pitch mixture was decanted from the coke. Next, the chloroform was evaporated by placing the mixture of coke and liquid in a pan for 3 hours. The pan was placed on an angle to allow excess liquid to drain from the coke. Calcining was carried out by placing the coke in an oven, increasing the temperature to 2600°F over a period of about 2.5 hours and thereafter maintaining the temperature at 2600°F for 2.0 hours.

### Example 2

Another sample of the same green coke was covered for 15 minutes by 720°F+ thermal tar heated to 200°F. After decanting the thermal tar, coke was placed on the sloped pan for 3 hours to remove excess liquid. Calcining was done as in Example 1.

### Example 3

Another sample of the same green coke was heated to roughly 330°F and then placed in a beaker with -60 mesh particles of 900°F+ solvent-solluble coal tar pitch. Mild shaking of the mixture caused pitch particles to adhere to the coke. Calcining again was carried out as in Example 1.

Physical properties of the coker feedstocks used in the examples are presented in Table 1. VBD and CTE of cokes produced in Examples 1-3 and a base case, where no coker feed was added, are presented in Table 2.

It is apparent from the data that soaking the green coke with coker feedstock increases the density of the calcined coke. The CTE of the calcined coke however was somewhat increased in the process. The amount of coker feedstock consumed in the process varied from about 7 to 10 percent based on the green coke.

The process of the invention has been described in its application to premium coke. However, it also can be used with other grades of coke. For example, large quantities of coke are produced for use in electrodes consumed in the manufacture of aluminum. This "aluminum grade" coke is distinguished from premium coke in its lack of the needle-like structure which denominates premium coke. While CTE is not a factor in the characterization of regular or aluminum grade coke higher coke density is desirable for such coke when it is used in the manufacture of electrodes.

Aluminum grade coke is also prepared by delayed coking and calcining under much the same conditions as are used in premium coking. Highly aromatic feedstocks are not required, usually such coke is prepared from resids or other heavy hydrocarbon fractions. Again, when aluminum grade coke is used in carrying out the invention the feedstock employed to contact the green coke may be the same feedstock used in making the coke or it may be a different feedstock.

## Claims

1. A process for increasing the density of calcined coke which comprises contacting green (uncalcined) coke with a coker feedstock and thereafter calcining said coke.

2. A process as claimed in claim 1 in which the coke is aluminum grade coke.

3. A process for increasing the density of calcined premium coke which comprises contacting green (uncalcined) premium coke with a coker feedstock and thereafter calcining said coke.

4. A process as claimed in any one of claims 1 to 3 in which the coker feedstock is a portion of the same feedstock used in the preparation of the green coke.

5. A process as claimed in any one of claims 1 to 3 in which the coker feedstock is a different feedstock from that used to prepare the green coke.

6. A process as claimed in any one of the preceding claims in which the green coke is passed through a bath of liquid coker feedstock.

7. A process as claimed in any one of claims 1 to 5 in which the green coke is sprayed with liquid coker feedstock.

8. A process as claimed in any one of claims 1 to 5 in which the green coke is passed through a finely divided feedstock powder.

9. A premium coking process which comprises heating an aromatic mineral oil feedstock to an elevated temperature, introducing the heated feedstock over a period of time into a coking drum under delayed coking conditions wherein the heated feedstock soaks in its contained heat to convert the feedstock to cracked vapors and premium coke, removing coke from the coke drum upon completion of the delayed coking, cooling the coke, contacting the cool coke with a portion of the aromatic mineral oil feedstock, and calcining the contacted coke to obtain calcined premium coke of increased density.

10. A premium coking process which comprises heating an aromatic mineral oil feedstock to between about 850°F and about 1100°F, introducing the heated feedstock over a period of time into a coking drum wherein the heated feedstock soaks in its contained heat at a temperature between about 800°F and about 1000°F and a pressure between about 15 psig and about 200 psig which is sufficient to convert the feedstock to cracked vapors and premium coke, removing coke from the coke drum upon completion of the coking with a high velocity jet of water, contacting the removed coke with a portion of the aromatic mineral oil feedstock and calcining the contacted coke at a temperature between about 2000°F and about 3000°F for between about one half hour and about ten hours to obtain calcined premium coke of increased density.

11. A process as claimed in claim 9 or claim 10 in which the removed coke is passed through a liquid bath of the aromatic mineral oil feedstock.

12. A process as claimed in claim 9 or claim 10 in which the removed coke is sprayed with liquid aromatic mineral oil feedstock.

13. A process as claimed in claim 9 or claim 10 in which the aromatic mineral oil feedstock is a solid at the contacting temperature and the removed coke is passed through a finely divided powder of such feedstock.

14. A process as claimed in any one of claims 9 to 13 in which the aromatic mineral oil feedstock is selected from the group consisting of thermal tar, decant oil, pyrolysis tar and pitch.
